

## UNITED STATES PATENT OFFICE

1,946,141

## WRAPPING PAPER

Walter W. Herrick, Milford, N. J., assignor to  
 Riegel Paper Corporation, Riegelsville, N. J.,  
 a corporation of New Jersey

No Drawing. Application April 1, 1932  
 Serial No. 602,633

6 Claims. (Cl. 92—21)

This invention relates to a heat-sealable opaque waxed paper for wrapping food-stuffs, and, more particularly, bread, cake, and the like.

The paper commonly used for the purpose is 5 a sulphite or glassine sheet which as a rule has no loading, although this old wrapping sheet has in certain cases been replaced by a similar sulphite sheet having a coating of casein or the like in combination with clay, talc, and similar 10 materials, with printing in color applied thereto on one side of the sheet, and then an outer film of paraffin wax.

I have discovered that by loading the paper, either sulphite or glassine, with titanium dioxide, 15 I can produce a waxed wrapping sheet which not only is of a purer white color, giving an appearance of cleanliness of particular value in wrappers of this type and at the same time increasing the brilliance of the matter printed in color 20 thereon, but also, and what is of more importance, has an improved sealing quality—that is to say, the seal produced by the application of heat is more secure and hence is less likely to be pulled apart than that obtained with a waxed paper 25 coated as heretofore, particularly when the coating film is thick enough to give the paper the desired degree of opacity.

What I claim as new, and desire to secure by Letters Patent, is—

30 1. As a new article of manufacture, a heat-

sealable opaque wrapping paper for food stuffs loaded with titanium dioxide and with a coating of wax applied directly to one or both sides thereof.

2. A heat-sealable opaque wrapping for food 60 stuffs comprising a sheet of paper loaded with titanium dioxide to give it the desired whiteness and opacity and with matter printed on one side thereof and a coating of wax applied directly 65 thereto over the printed matter.

3. A heat-sealable opaque wrapping for bread and the like comprising a sheet of sulphite paper loaded with titanium dioxide and coated with wax.

4. A heat-sealable opaque wrapping for bread 70 and the like comprising a sheet of glassine paper loaded with titanium dioxide and coated with wax.

5. A heat-sealable opaque wrapping for food 75 stuffs comprising a sheet of sulphite paper loaded with titanium dioxide and with a coating of wax applied directly to one or both sides thereof.

6. A heat-sealable opaque wrapping for bread 80 and the like comprising a sheet of sulphite paper loaded with titanium dioxide to give it the desired whiteness and opacity and with matter printed in color on one side thereof and a coating of wax applied directly thereto over the printed matter.

WALTER W. HERRICK. 85

35

40

45

50

105

55

110